

1

3,749,552  
SIMULTANEOUS INTRODUCTION OF QUATERNARY AMMONIUM SALT RESIDUES AND SULFONE RESIDUES INTO FIBROUS CELLULOSE  
Stanley P. Rowland, New Orleans, La., assignor to the United States of America as represented by the Secretary of Agriculture  
No Drawing. Filed Dec. 9, 1970, Ser. No. 96,608  
Int. Cl. D06m 13/28, 13/46  
U.S. Cl. 8—188

1 Claim 10

## ABSTRACT OF THE DISCLOSURE

This invention relates to a process for the introduction of quaternary ammonium salt residues and sulfone residues into fibrous cellulose. More particularly, this invention relates to a process for the simultaneous introduction of quaternary ammonium salt residues and sulfone residues into fibrous cellulose.

A non-exclusive, irrevocable, royalty-free license in the invention herein described, throughout the world for all purposes of the United States Government, with the power to grant sublicenses for such purposes, is hereby granted to the Government of the United States of America.

An object of this invention is to provide a simple and practical process for the preparation of cotton fabrics containing substituents bearing quaternary ammonium salt groups and crosslinks derived from divinyl sulfone and "precursors" of divinyl sulfone. A further object of this invention is to prepare a cotton fabric which fabric has "built-in" catalysts for the thermal reversibility of crosslinkages derived from divinyl sulfone and "precursors" of divinyl sulfone.

It has been found that quaternary ammonium groups attached via different substituent linkages to cotton cellulose act as internal catalysts for the thermal reversibility of crosslinkages derived from divinyl sulfone. For effective introduction and removal of creases, the quaternary ammonium group is converted to the acetate salt form, and as such it provides catalysis at normal ironing temperatures without causing instability at conventional usage temperatures of conventional laundering and drying conditions. Details are described in the publication "Introduction and Removal of Durable Creases from Wrinkle-Resistant Cotton Fabrics" [Text. Res. J. 40, 607 (1979)].

The cotton fabrics which contain quaternary ammonium groups and sulfone residues and which are the basis for the study referred to in the above manuscript were prepared as follows:

## COMPOSITION, TYPE 1

- (a)  $(CH_3)_3NCH_2CHOHCH_2$ —substituents were introduced into cotton fabric.
- (b) The tertiary-amino groups were quaternized by reaction of the DEAE-cotton with methyl iodide.
- (c) The quaternary ammonium cotton ("Quat 1") was converted to the base form by treatment with dilute NaOH, followed by extensive rinsing.
- (d) The base form of Quat 1 was contacted with a solution of divinyl sulfone and allowed to react for 60 minutes at room temperature, or it was given a back-cure for 10 minutes at 140° C.

2

Details are described in the publication "A Delayed Curing Cotton Fabric Based on an Internally Catalyzed Cotton Cellulose and Divinyl Sulfone" [Text. Res. J. 39, 173 (1969)].

## COMPOSITION, TYPE 2

- (a)  $(CH_3)_3NCH_2CHOHCH_2$ —substituents were introduced into cotton fabric.
- (b) The substituted cotton from (a) just above with the quaternary groups in the base form was reacted with divinyl sulfone in the same manner as described for the preceding composition.

This is described in detail in the publication "Variations in a Delayed-Curing Cotton Fabric Based on Internal Catalysis and Divinyl Sulfone" [Text. Res. J. 40, 101 (1970)].

It has now been found that the quaternary ammonium substituent groups and the divinyl sulfone residues can be introduced into cotton simultaneously in a single operation. The compositions which result are essentially the same as those described above under the heading, "Composition, type 2." The compositions of type 2 as prepared by the method described above (which is that of application Ser. No. 765,613 filed Oct. 7, 1968, now U.S. Pat. No. 3,574,522.) could not be prepared from the more common precursors for divinyl sulfone since these require two moles of base to generate the divinyl sulfone, in addition to catalytic amounts of base for catalysis. The current invention is applicable to all of these divinyl sulfone generators which were not appropriate for the preceding case: e.g., bis(2-chloroethyl) sulfone (and corresponding bromo- and iodo compounds), bis(pyridinium-ethyl) sulfone dichloride, disodium bis(2-sulfatoethyl) sulfone, and disodium bis(2-thiosulfatoethyl) sulfone.

The following examples illustrate but do not limit the scope of this invention.

## Example 1

A solution was prepared from 11.8 g. of divinyl sulfone, 18.8 g. of 3-chloro-2-hydroxypropyltrimethylammonium chloride, and 13.8 g. of potassium carbonate in 55.4 g. of water. Cotton fabric (80 x 80 printcloth, desized, scoured, bleached) was padded through this solution. The wet pickup was about 110%. The wet fabric was cured in a forced draft oven for 11 minutes at 140° C. The fabric was rinsed thoroughly in warm running tap water, in dilute acetic acid, and finally in distilled water. After drying at room temperature, the fabric showed a 4% increase in weight over that of the initial weight. The nitrogen content was 0.32% and the sulfur content was 0.89%. This corresponds to a ratio of gram atoms of sulfur:nitrogen of 1.22. The ratio may be varied over a wide range by altering the initial weight ratio of the reagents in the pad bath.

## Example 2

The process described above was conducted with 11.8 g. of bis(2-hydroxyethyl) sulfone in place of the divinyl sulfone. The major difference in the product from that above was a sulfur content of 0.25% and a ratio of gram atoms of sulfur:nitrogen of 0.34.

## Example 3

$CH_3OCH_2CH_2SO_2CH_2CH_2OCH_3$  was employed in place of divinyl sulfone in Example 1, with the addition of 10

g. of dimethyl sulfoxide to the solution. The product contained 0.3% nitrogen and 0.3% sulfur. Higher levels of nitrogen and sulfur were incorporated by conducting the cure at 180° C. for 3 minutes.

Example 4

The process of Example 1 was carried out with 15 g. of  $\text{HOCH}_2\text{OCH}_2\text{CH}_2\text{SO}_2\text{CH}=\text{CH}_2$  (the product from reaction of one mole of formaldehyde with one mole of divinyl sulfone; refer to U.S. Pat. 3,202,474) in place of the divinyl sulfone. The nitrogen content of the fabric was 0.3% and the sulfur content was 0.65%.

Example 5

Reactions conducted as those described in Examples 1, 2, 3, and 4 but by replacing (wt. for wt.) the 3-chloro-2-hydroxypropyltrimethylammonium chloride with glycidyltrimethylammonium chloride and by using potassium carbonate, sodium carbonate, or mixtures of sodium carbonate and sodium bicarbonate for catalysis yielded generally similar results; in most cases, however, the nitrogen introduced into the fabric was approximately 25% or more higher than the values described above.

Example 6

To 11.8 g. of divinyl sulfone in 69.4 g. of water was added 18.8 g. of 3-chloro-2-hydroxypropyltrimethylammonium chloride. A sample of cotton printcloth was padded thoroughly in this solution and then it was immersed in a 6% solution of NaOH for 2½ hours at room temperature. Following rinsing and drying as described for Example 1, there was observed a 9% increase in weight of the fabric. The nitrogen content was 0.17% and the sulfur content was 2.07%. The ratio of gram atoms of sulfur:nitrogen was 3.15. Potassium hydroxide is essentially equivalent to sodium hydroxide in this reaction.

Example 7

The procedure of Example 6 was conducted with 15 g. of glycidyltrimethylammonium chloride in place of the 3-chloro-2-hydroxypropyltrimethylammonium chloride and with 23% sodium hydroxide solution in place of the 6% solution. The cotton fabric which resulted from this reaction contained 0.43% nitrogen and 2.0% sulfur. The cellulose was converted to lattice II structure (as evidenced from X-ray diffractograms) in this case. All preceding products showed lattice I structure.

Example 8

In the manner of Example 7, separate reactions were carried out by replacing the divinyl sulfone with 15 g. of bis(2-pyridylethyl) sulfone dichloride, disodium bis(2-sulfatoethyl) sulfone, or disodium bis(2-thiosulfatoethyl) sulfone. The resulting chemically modified cotton fabrics contained about 0.25% nitrogen and the sulfur contents ranged between 2 and 3%.

Example 9

Cotton fabric was padded into 15.0 g. of bis(2-chloroethyl) sulfone and 15.0 g. of glycidyltrimethylammonium chloride in 69.4 g. of dioxane-water and the wet fabric was padded through a 12% solution of NaOH. The fabric was stored wet for 2 hours and then rinsed thoroughly in water, dilute acetic acid, and finally, water. The product fabric contained 0.2% nitrogen and 2.0% sulfur.

Example 10

Cotton printcloth was padded into a solution of divinyl sulfone (10%) and glycidyltrimethylammonium chloride (10%) to a wet pickup of approximately 120%. The wet fabric was spread flat in an enamel pan and covered with a solution of NaOH which was just sufficient to contact the entire fabric. The solution contained an amount of NaOH (about 3.2 g.) equivalent in moles to the glycidyltrimethylammonium chloride on 100 g. of the fabric. The fabric was continued in contact with the aque-

ous alkali for 3 hours at room temperature, after which it was rinsed and dried as previously described. The nitrogen and sulfur contents of the fabric were 0.3 and 1.5%.

Example 11

With bis(2-hydroxyethyl) sulfone or the product from reaction of 2 moles of formaldehyde with 1 mole of divinyl sulfone (refer to U.S. Pat. No. 3,202,474) replacing the divinyl sulfone of Example 10 (wt. for wt.), little or no sulfur was introduced into the cotton unless the fabric was subjected to a drying and curing period in a forced draft oven at a temperature above about 80° C.

Example 12

Cotton fabric was padded in a solution of divinyl sulfone (11.8%) and 3-chloro-2-hydroxypropyltrimethylammonium chloride (19%) to about 120% wet pickup and then it was soaked in a solution containing NaOH (6%) and sodium sulfate (20%) for 2½ hours at room temperature. The final nitrogen and sulfur contents of the fabric were 0.18% and 3.54%.

General comments.—All of the chemically modified cotton fabrics described in the foregoing examples exhibited improvements in conditioned and wet wrinkle recovery angles over the values of the original cotton fabric (181° and 172°, respectively, for the conditioned and wet values [W+F] for the unmodified printcloth). These values for the chemically modified cottons appeared to be primarily dependent upon the concentration of the alkali employed in the reaction as well as the temperature of the cure and the specific nature and add-on of the sulfone reagent. Wet wrinkle recovery angles in the range of 250–300° are readily achieved under the conditions of reaction described above and in many cases conditioned wrinkle recovery angles in the same range are obtained (e.g., values of conditioned and wet wrinkle recovery angles of 252 and 277 for the product of Example 12).

These chemically modified cottons are valuable for their wrinkle resistant characteristics and for their amenability to introduction and removal of creases by ironing operations as previously described [Text. Res. J., 40, 607 (1970)].

We claim:

1. A process of modifying a cellulosic fabric which comprises:

- (a) padding a cellulosic fabric in an aqueous solution containing a 3-halo-2-hydroxypropyltrimethylammonium halide or glycidyltrimethylammonium chloride, a compound selected from the group consisting of divinyl sulfone and divinyl sulfone generators, and an alkali metal base selected from the group consisting of sodium carbonate, sodium bicarbonate, mixtures of sodium carbonate and sodium bicarbonate, and potassium carbonate,
- (b) curing the padded fabric from (a), and
- (c) washing the fabric from (b) free of excess reagents.

References Cited

UNITED STATES PATENTS

- |           |         |                        |          |
|-----------|---------|------------------------|----------|
| 3,106,439 | 10/1963 | Valentine et al. ----- | 8—DIG. 2 |
| 3,218,118 | 11/1965 | Steele et al. -----    | 8—120    |
| 3,574,522 | 4/1971  | Rowland et al. -----   | 8—116.2  |

FOREIGN PATENTS

- |           |        |                     |       |
|-----------|--------|---------------------|-------|
| 958,857   | 5/1964 | Great Britain ----- | 8—120 |
| 1,004,757 | 9/1965 | Great Britain ----- | 8—120 |

OTHER REFERENCES

- McKelvey et al.: American Dyestuff Reporter, vol. 49, No. 22, pp. 19–24, Oct. 31, 1960.  
 Berni et al.: American Dyestuff Reporter, pp. 29–35, June 7, 1965.

(Other references on following page)

## OTHER REFERENCES

- Tesoro et al.: Textile Research Journal, 31, 283-295 (1961).  
Soignet et al.: Textile Research Journal, 36, 978-989 (1966).  
Rowland et al.: Textile Research Journal, 40, 101-108 (1970).  
Soignet et al.: Journal of Applied Polymer Science, 13, 81-92 (1969).

GEORGE F. LESMES, Primary Examiner  
J. CANNON, Assistant Examiner  
5 U.S. CL. X.R.  
8-120, DIG. 2; 260-231 A